

## UNITED STATES PATENT OFFICE

2,638,413

## ABRASIVE ARTICLES

Norman P. Robie, Hamburg, N. Y., assignor to  
Electro Refractories & Abrasives Corporation, a  
corporation of Delaware

No Drawing. Application August 10, 1949,  
Serial No. 109,621

6 Claims. (Cl. 51-298)

1

This invention relates to abrasive articles and more particularly to grinding wheels bonded with thermo-setting resin.

A primary object of my invention is to produce abrasive bodies with superior cutting ability, which may be measured either in terms of work done per body during the useful life of the same, or in terms of rate of cut. Another object is to provide an abrasive wheel which is cooler during cutting than the usual wheels, particularly those bonded with synthetic resins capable of high speed operation. Another object is to increase the safety factor by reducing the tendency to break when the wheel is used in severe-cutting applications.

My invention resides particularly in the use of certain fillers which I have found it advantageous to incorporate in the mix from which the body or wheel is made. These fillers are not in themselves abrasives in the usual sense, but greatly improve the performance of the body or wheel when it is in operation by modifying and/or extending the binder used therein. The use of fillers in such wheels is old in the art, the use of such materials as cryolite, clay, fine alumina, lead oxide, flint, rouge, lime or magnesium oxide having been described in patents or practiced more or less widely in the industry. In some cases the selection of these materials has been to secure some chemical reaction with the resin or with the water vapor released during the curing operation. The use of lubricating fillers such as graphite has also been suggested.

The fillers according to my invention, are chemically inert and do not possess the quality of lubricity, hence they seem to fall into a different category from the foregoing. My fillers in common with some of the others, seem to make the abrasive articles or wheels containing them somewhat denser and harder than when the fillers are left out, but they vary sharply from the others, in that in spite of this action, they increase the speed of cut and decrease the heat of grinding. It is particularly important in the type of resin bonded wheels known as cutoff wheels that they be cool cutting and yet possess long service life. Otherwise these wheels not only burn and spoil the surface of the metal being cut, but the heat causes expansion or warping of either the wheel or the metal so that the wheel binds in the slot being cut, with the result that the wheel seizes and breaks. Further, if excessive heat is generated, the bond disintegrates, causing chips to break out of the wheel edge. To avoid these difficulties, such wheels are often made relatively open or porous, which weakens the same with the result that they wear

2

away very rapidly. I have found that by the use of my invention it is possible to make the wheels far stronger and more solid, and yet not secure excessive heating even when metal is removed at a rapid rate. While my invention is highly applicable to cutoff wheels, it is not limited to them, but is rather applicable to resin bonded wheels and abrasive articles of all sorts.

I have found that certain lead salts which are not reactive with phenolic resins and do not form lead phenolates, as do those suggested by Kuzmick in U. S. Patent #2,083,719, are unusually valuable fillers in phenolic resin bonded abrasives. These salts are the substantially insoluble and anhydrous lead salts of strong acids, including specifically lead chloride, lead fluoride, lead sulfate, lead fluo-chloride and the like. I do not know why these fillers are so superior, but I have established by repeated tests in the laboratory and in the field that such is the case. I also know that they do not embrittle the resin by reaction therewith, as do oxidic compounds of lead.

In the manufacture of abrasive articles in accordance with my invention, I have used my fillers in various amounts from as low as 3% of the mix by weight to as high as 30%. I prefer, however, to use from 10 to 25% with 20% as generally satisfactory.

The abrasive employed may be of any desired type, such as aluminum oxide, corundum, emery, diamonds and the like. The binder may be of any thermo-setting resin of the type commonly used as binders in the abrasive industry such, for example, as phenolic or alkyd resins. I preferably employ a finely powdered, less than 1% on 100 mesh, less than 15% on 325 mesh, initially fusible and soluble, heat reactive, heat hardening phenol-formaldehyde resin capable of heat hardening into an infusible, insoluble state. The phenol-formaldehyde resin is a two stage resin containing usually hexamethylenetetramine ground therein to act as a hardening agent.

Preferably I use a plasticizer, which may be a solvent, a liquid resin or a solution of resin in accordance with the well known practice in the abrasive industry. The following may be employed; cresol, furfuryl alcohol, furfural, liquid phenolic resins.

These materials are thoroughly mixed according to conventional practice and formed into articles of desired shapes by either hot or cold pressing, and the articles may be completely cured during hot pressing, or the formed articles may be heated or oven-baked in the usual manner to thermo-set the bond.

In order that the method of manufacture may

be clearly understood, I give the following examples by way of illustration and not limitation:

*Example I*

200 grams of technical grade, finely powdered lead chloride is first mixed dry with 110 grams of powdered phenol formaldehyde resin of the A stage heat reactive variety (sold by the Varicun Chemical Corporation under the number V1364). In a separate container I mix together 690 grams of fused alumina oxide abrasive grains using equal amounts of grits 24, 30 and 36 respectively. After these are well mixed, they are wet up with 8 cc. of cresol and the mixture of powdered bond and filler is then added and thoroughly mixed in. The material thus prepared is then placed in a mold, levelled and pressed in the manner well known to the art, after which it is removed from the mold and baked or cured, again in the manner familiar to the art, in this case by gradually raising the temperature to 360° F. over a period of five hours and holding it at that temperature for at least twenty-four hours, after which the article is removed from the oven and finished in the usual manner.

*Example II*

A wheel in which silicon carbide is used as the abrasive may be made by employing the following percentages of ingredients by weight:

Silicon carbide grain 64.4%. The grain may be in the 24, 30 and 36 grain size, and preferably equal quantities of each size are used.

The bonding agent may be the same as specified in Example I, and constitutes 12.6% of the final product.

Lead sulfate in powdered form is employed to the extent of 23% of the weight of the final product.

The silicon carbide grain is wetted with a suitable plasticizer, for example 30 cc. of cresol per pound of resin bond used, before mixing with the lead sulfate filler and the resin powders. The material is then molded to a density of about .0891 pound per cubic inch and may then be cured or baked as described in Example I.

The specific examples I have given have been concerned chiefly with cutoff wheels because due to their thinness, these can be tested with minimum requirement for material. I do not confine my use of my fillers to such wheels however, but may use them in portable wheels, snagging wheels, thread grinding wheels, or any other type of abrasive in which synthetic resin bonds are used. Their use in wheels containing natural or synthetic rubber in the bond is beneficial. The fillers may be used with any of the common types of abrasive including alumina or silicon carbide, and with phenolic, alkyd or other thermosetting resins. Their use is beneficial without regard to the type of plasticizer used. The wheels may be made by either hot or cold pressing methods.

I may admix my fillers with other cheaper fillers, such as cryolite or lime in order to extend their utility, or I may use them unmixed. I have in general used them in powder form such that 100% will pass through a 325 mesh sieve, but their beneficial effect is not primarily dependent upon size so long as they are of the order of fineness of 100 mesh or less.

In a series of comparative tests, I made wheels identical with one another except for the filler used, as follows: a mix was made from 79% by weight of fused alumina grain comprising equal proportions of 24, 30 and 36 grit. This grain was

wet up with a plasticizer in the usual way and a premixed lot of powder consisting of 14.2% by weight of reactive heat-hardenable phenolic resin, 5.9% filler and 0.87% lime was then mixed in and the mix formed into wheels having a density of 0.0866 pound per cubic inch. These wheels were then baked between batts, their temperature being raised to 360° F. and held at that temperature for over nine hours. The wheels, each of which was 16 x 1/8 x 1 inches were then used to make 25 cuts through a 1 inch bar of cold rolled steel and the loss of abrasive determined by weighing the wheel before and after use. My lead fluoride filler gave superior results as follows:

|    | Filler                    | Grams Wheel Loss |
|----|---------------------------|------------------|
| 20 | Lead fluoride.....        | 32               |
|    | Cryolite.....             | 36               |
|    | Potassium fluoborate..... | 40               |

The other fillers here chosen are those commonly used in such abrasive articles. It is known that their effectiveness decreases as the percentage falls below that used, so that if for instance the volume of the cryolite and fluoborate had been as small as the volume of the much denser lead salt, the results would have been even more favorable to my material.

In another series of comparative tests made with my fillers in comparison with litharge, 69% by weight of fused alumina grain, sized as above, was similarly made up into wheels using 11% of powdered resin and 20% by weight of filler. The wheels in this case were each pressed to a density of 0.11 pound per cubic inch. After baking, they were each used to make ten cuts through 1 1/4 inch stainless steel rods and the loss of weight of each wheel measured as before. The results are given below:

|    | Filler                                             | Grams Wheel Loss |
|----|----------------------------------------------------|------------------|
| 45 | Lead chloride, C. P.....                           | 10               |
|    | Lead chloride, technical.....                      | 9                |
|    | Lead sulfate, C. P.....                            | 10.5             |
|    | Litharge, technical.....                           | 18.5             |
| 50 | Basic lead sulfate (Pb SO <sub>4</sub> ; PbO)..... | 19               |

Still further tests were made under drastic test conditions, in which it was attempted to cut slices from a tough four inch square stainless steel bar. The wheels made with conventional fillers made only partial cuts and then, because of the tremendous heat generated, seized or stuck, crumbled and broke. With wheels made using my lead chloride and lead sulfate fillers, complete cuts were readily made when the wheels were applied with the same pressure by means of a hydraulic feed piston. A litharge filled wheel also made a full cut but lost much more weight, as shown in the following table.

|    | Filler                                                | Grams Wheel Loss |
|----|-------------------------------------------------------|------------------|
| 65 | Litharge.....                                         | 169              |
| 70 | PbCl <sub>2</sub> .....                               | 57               |
|    | 1/2 PbCl <sub>2</sub> and 1/2 PbSO <sub>4</sub> ..... | 51               |
|    | PbSO <sub>4</sub> .....                               | 46               |

Commercial field trials in which wheels with my fillers have been used in comparison with others on the market have confirmed these lab-

oratory results, with superiority in pieces processed per wheel running 50% above normal in many instances.

Having thus described my invention in general terms and given a specific example of its application, I desire patent protection within the scope of the following claims:

1. A cutoff wheel comprising abrasive grains, from 10% to 25% by weight of an anhydrous lead salt of a strong acid selected from a group consisting of non-basic lead sulfate, a lead halide and mixtures thereof, and a thermo-set phenolic resin bond uniting said grains and said lead salt into an integral body, said lead salt being substantially insoluble in water and non-reactive with said bond and being substantially uniformly dispersed throughout said body.

2. As an intermediate article of manufacture, a shaped object for the manufacture of an abrasive body therefrom, said shaped object consisting of a compacted formed mixture of abrasive granules, a thermal setting phenol formaldehyde resin, and from 3% to 30% by weight of a finely divided lead salt of a strong acid, said salt being substantially insoluble in water and non-reactive with said bond and being a member of the group of compounds consisting of non-basic lead sulfate, lead halides and mixtures thereof.

3. An abrasive article comprising abrasive grains, an anhydrous lead salt of a strong acid in finely divided form, said salt being a member of the group consisting of non-basic lead sulfate, lead halides and mixtures thereof, and a phenolic resin thermo-set bond uniting said grains and said lead salt into an integral body, said lead salt being substantially insoluble in water and non-reactive with said bond and being substantially uniformly dispersed throughout said body, said

lead salt comprising from 3% to 30% by weight of the article.

4. An abrasive article comprising abrasive grains, an anhydrous lead salt of a strong acid in finely divided form, said salt being a member of the group consisting of non-basic lead sulfate, lead halides and mixtures thereof, and a phenolic resin thermo-set bond uniting said grains and said lead salt into an integral body, said lead salt being substantially insoluble in water and non-reactive with said bond and being substantially uniformly dispersed throughout said body, said lead salt comprising from 10% to 25% by weight of the article.

15 5. An abrasive article comprising abrasive grains, from 3% to 30% by weight of a lead halide in finely divided form and a phenolic resin thermo-set bond uniting said grains and said lead salt into an integral body, the lead salt being substantially uniformly dispersed throughout said body.

20 6. An abrasive article comprising abrasive grains, from 3% to 30% by weight of a non-basic lead sulfate in finely divided form and a phenolic resin thermo-set bond uniting said grains and said lead salt into an integral body, the lead salt being substantially uniformly dispersed throughout said body.

NORMAN P. ROBIE.

References Cited in the file of this patent

UNITED STATES PATENTS

| Number    | Name                 | Date          |
|-----------|----------------------|---------------|
| 2,083,719 | Kuzmick et al. ----- | June 15, 1937 |
| 2,273,891 | Pollak et al. -----  | Feb. 24, 1942 |
| 2,456,920 | Coes -----           | Dec. 21, 1948 |